# EUROPEAN PATENT SPECIFICATION

(11) **EP 0 228 801 B1**
(45) Date of publication and mention of the grant of the patent: **02.01.1991**
(21) Application number: 86308989.2
(22) Date of filing: 18.11.1986
(51) Int. Cl.: D21H 17/33

(54) **Aqueous dispersed solution of substituted succinic anhydride**
Dispergierte wässrige Lösung eines substituierten Bernsteinsäureanhydrids
Solution aqueuse dispersée d'un anhydride succinique substitué

(30) Priority: 18.11.1985 JP 258292/85
(43) Date of publication of application: 15.07.1987
(73) Proprietor: SEIKO KAGAKU KOGYO CO., LTD., Akashi-shi Hyogo 673 (JP); HOKUETSU PAPER MILLS, LTD., Nagaoka-shi Niigata-ken 940 (JP); NIPPON OIL CO. LTD., Minato-ku Tokyo (JP)
(72) Inventor: Yoshioka, Shigehiko, Akashi-Shi Hyogo (JP); Yamada, Hideto, Akashi-Shi Hyogo (JP); Yata, Akihiro, Nagaoka-Shi Niigata (JP); Sato, Hisatake, Yokohama-Shi Kanagawa (JP)
(74) Representative: Heath, Derek James

(56) References cited:
- EP-A- 0 151 646
- EP-A- 0 177 260
- US-A- 4 533 434
- ABSTRACT BULLETIN OF THE INSTITUTE OF PAPER CHEMISTRY, vol. 55, no. 2, August 1984, pages 245,246, abstract no. 2297, Appleton, Wisconsin, US; & JP-A-91 897/83 (KANZAKI PAPER MFG. CO. LTD; ARAKAWA CHEMICAL INDUSTRY LTD) 31-05-1983
- ABSTRACT BULLETIN OF THE INSTITUTE OF PAPER CHEMISTRY, vol. 54, no. 11, May 1984, page 1340, abstract no. 12666, Appleton, Wisconsin, US; & JP-A-60 095/83 (ARAKAWA CHEMICAL INDUSTRY LTD) 09-04-1983
- ABSTRACT BULLETIN OF THE INSTITUTE OF PAPER CHEMISTRY, vol. 54, no. 3, September 1983, page 350, abstract no. 3226, Appleton, Wisconsin, US; & JP-A-143 600/82 (ARAKAWA CHEMICAL INDUSTRY LTD) 04-09-1982

## Description

The present invention relates to an aqueous dispersed solution of a substituted succinic anhydride. More particularly, the present invention relates to such an aqueous dispersion of a substituted succinic anhydride used as a sizing agent having excellent sizing effect and preferable operability in paper making steps and exhibiting excellent operations even in a dilute stability.

There is known a sizing paper employing an aqueous dispersed solution of a substituted succinic anhydride, and various types of aqueous dispersions have been heretofore proposed such as, for example, an aqueous dispersion prepared by mixing an aqueous solution of cationic starch and a substituted succinic anhydride by a strong mechanical agitation in a homogeneous state (disclosed in Japanese Patent Publication No. 2305/1964 official gazette), an aqueous dispersion prepared by dispersing a substituted succinic anhydride in water or an aqueous solution of specific aqueous soluble polymer substance with the aid of a selected surfactant (disclosed in Japanese Patent Publication No. 36044/1978 official gazette, Japanese Patent Laid-open No. 45731/1983 official gazette, Japanese Patent Laid-open No. 47498/1984 official gazette), and further an aqueous dispersion prepared by dispersing a substituted alkyl-substituted or alkenyl-substituted succinic anhydride or a mixture (a) of the succinic anhydrides which contain 70 to 99.9 percent by weight and a mixture (b) of polyoxyethylene alkyl-ether phosphoric acid ester, polyoxyethylene alkylaryl ether phosphoric acid ester or the mixture of these phosphoric acid esters which contain 0.1 to 30 percent by weight in water with the aid of an aqueous solution of aqueous soluble polymer compound (disclosed in Japanese Patent Laid-open No. 28598/1985).

However, in the abovementioned aqueous dispersion employing the former cationic starch of the aqueous dispersions of the substituted succinic anhydrides, a considerably large apparatus is not only required to disperse the substituted succinic anhydride in water, but it is difficult to sufficiently pulverize the aqueous dispersed solution thus obtained into fine dispersion particles, and the resultant dispersion has such a disadvantage that the dispersion cannot avoid the slight decrease in the sizing performance.

In the above-described aqueous dispersion employing the latter mixture of the aid, the prepared mixture loses its stability in preservation and cannot secure a sufficient dispersibility of the substituted succinic anhydride in water, and the resultant aqueous dispersion not only loses its sizing effect with a lapse of time after preparation but deteriorates in the dispersibility of the substituted succinic anhydride having an internal olefin structure adapted for a sizing agent in water. Incidentally, a process for producing an aqueous dispersed solution by the prepared mixture has drawbacks such that, if the prepared mixture is dispersed in the aqueous solution dissolved in advance in a cationic starch when the aqueous dispersed solution is prepared from the prepared mixture, an aqueous dispersed solution having prefereble dilute stability can be produced, but since the aqueous solution itself of the cationic starch is unstable in an ageing manner, the cationic starch must be dissolved in water immediately before using the aqueous dispersed solution as a sizing agent, and since the underwater dispersibility for the substituted succinic anhydrides of the cationic starch is low, a strong (large-scale) emulsifying apparatus for preparing the aqueous dispersed solution is required.

Further, the aqueous dispersion utilizing the substituted-alkyl succinic anhydride or substituted-alkenyl succinic anhydride or a mixture (a) of the succinic anhydrides which contain 70 to 99.9 percent by weight and a mixture (b) of polyoxyethylene alkyl-ether phosphoric acid ester, polyoxyethylene alkylaryl ether phosphoric acid ester or the mixture of these phosphoric acid esters which contain 0.1 to 30 percent by weight in water with the aid of an aqueous solution of aqueous solution polymer compound, and the resultant aqueous dispersion further provides preferable dispersibility in water for the substituted succinic anhydride having an internal olefin structure as a sizing agent as its merits, but when the aqueous dispersion obtained from this mixture is used as a sizing agent in an industrual scale, some problems are still retained. In other words, the aqueous dispersion of the substituted succinic anhydride obtained from the mixture proposed in Japanese Patent Laid-open No. 28598/1985 exhibits dilute stability of the aqueous dispersion in the case where the cationic starch dissolved in water of continuous state is contained in the aqueous dispersion, but, in other cases, causes insufficient dilute stability, and when this aqueous dispersion is employed as a sizing agent in the practical paper making process, the dispersion has such a drawback that it contaminates the wires, rolls and other parts of the paper making machine and cannot operate continuously for a long period of time.

Therefore, the inventors of the present invention have discovered the fact that the aqueous dispersed solution of the substituted succinic anhydrides which contained specific aqueous soluble copolymer obtained with (meth)acrylic amide and N,N-dialkylaminoalkyl(meth)acrylamide as indispensable monomer ingredients could eliminate the various types of drawbacks with the aqueous dispersed solution described above, and has proposed the aqueous dispersed solution of the substituted succinic anhydrides which contained the specific aqueous copolymer, but have discovered other drawbacks in the operation that, when the aqueous dispersed solution of the substituted succinic anhydrides was utilized as a paper making sizing agent, the sizing effect in the low content addition range of the sizing agent was not always satisfactory, and, when applied to the acidic paper making step which did not use calcium carbonate filler and neutral paper making step of middle quality paper frequently produced by adding small amount of sulfuric acid band by using calcium carbonate filler, the separation of wet paper and rolls was deteriorated to cause the paper to be cut.

Accordingly, an object of the present invention is to provide an aqueous dispersed solution of a substituted succinic anhydride which can perform the operation of the aqueous dispersed solution of a substituted succinic anhydride which contained a specific aqueous soluble copolymer produced with the (meth)acrylamide and N,N-dialkylaminoalkyl(meth)acrylamide as indispensable monomer ingredients, i.e., the operation of excellent sizing effect and preferable dilute stability of the aqueous dispersed solution in paper making steps as well as perform a sizing effect sufficiently satisfied in a low content sizing agent addition range and achieve the entirely similar excellent operability to the other cases even in an acidic paper making step without using calcium carbonate filler and in a neutral paper making step, including the case where sulfuric acid is used.

With this object in view, the present invention is directed to an aqueous dispersion of a substituted succinic anhydride comprising an aqueous soluble copolymer - or a mixture monomer ingredient in an aqueous solution copolymer - which has 50 per cent or more by mol of (meth)acrylamide, 1 per cent or more by mol of N,N-dialkylaminoalkyl(meth)acrylamide, and a quantity of (meth)acrylic acid, characterised in that the first-mentioned copolymer or the mixture monomer ingredient has up to 98.5 per cent by mol of (meth)acrylamide, up to 49.5 per cent by mol of N,N-dialkylaminoalkyl(meth)acrylamide, and from 0.5 to 20 per cent by mol of (meth)acrylic acid.

In order to differentiate the two copolymers mentioned above, the first-mentioned copolymer is designated "A," in what follows while the second-mentioned copolymer is designated IIA2".

Preferred characteristics of the dispersion are set forth in claims 2-7.

EP-A-0 177 260, which was published after the priority date of the present Application, describes an aqueous dispersed solution of a substituted succinic anhydride which can contain (meth)acrylic acid as an optional ingredient. However, this particular acid is merely one of very many optional ingredients mentioned in that prior document and there is no suggestion there that it has any beneficial effect, nor is there any indication as to the amount of (meth)acrylic acid to be included in the dispersion.

The substituted succinic anhydrides in the aqueous dispersed solution of the substituted succinic anhydride according to the present invention can employ all of the known substituted succinic anhydrides used heretofore as a sizing agent, and more particularly comprise those substituted succinic anhydrides which contain hydrophobic hydrocarbon groups each having at least 8 and more preferably 12 to 36 carbon atoms such as substituted succinic anhydrides (having alkyl or alkenyl groups). Generally, the substituted succinic anhydrides comprise those feasibly produced by addition reaction of alpha-olefins, inner olefins or olefins of the mixture of them and maleic anhydride. Typically, when the substituted succinic anhydrides are, for example, octadecen-9, tetradecen-7, hexadecen-7, eicosene-11 or the mixture thereof; inner olefin selected from straight-chain internal inner olefin mixture having double bonds produced by the dehydrogenation reaction of straight-chain paraffin are distributed substantially uniformly at the respective positions except alpha-positions; and straight-chain inner olefin mixture having 70 percent or more by weight of total amount of inner olefins disposed at 2-, 3- and 4-positions of double bonds produced by anisotropic reaction of straight-chain alpha-olefin in the presence of catalyst; and the mixture produced by addition reaction of the anhydrides and maleic anhydride, i.e., when the substituted succinic anhydrides are those of alkenyl succinic anhydride having succinyl group in the substituted group, the sizing effect performed by the application of the substituted succinic anhydride of the present invention to the sizing agent for making paper in the paper making process is further improved.

The monomer ingredients of the aqueous soluble copolymer (A,) or (A₂) used together with the substituted succinic anhydrides in the aqeuous dispersed solution of the substituted succinic anhydrides are acrylamide, methacrylamide or both of them, i.e., (meth)acrylamide (a), N,N-dialkylamino.alkyl- acrylamide, N,N-dialkylamino.alkylmethacrylamide (b), acrylic acid, methacrylic acid or both of them, i.e., N,N-dialkylamino.alkyl(meth)acrylamide (b), i.e., (meth)acrylic acid (c). Incidentally, the N,N-dialkyl- amino.alkyl(meth)acrylamide (b) is basic third class amino group containing monomer represented by the following general formula where, in the formula, R is a hydrogen or methyl group, R₁ and R₂ represent a methyl group, ethyl group or propyl group, and n represents an integer of 2 to 4.

The aqueous soluble copolymer (A₁) can be readily produced by the ordinary polymerization of the monomer ingredients prepared at the abovementioned ratio of the compositions, but it is confirmed that the copolymner (A,) of 75 to 94 percent by mol of the (meth)acrylamide (a), 5 to 20 percent by mol of N,N-dialkylaminoalkyl(meth)acrylamide (b), and 1 to 10 percent by mol of (meth)acrylic acid (c) obtains more preferable results by the sizing effect in the low sizing agent addition range of the quality of the case using the aqueous dispersed solution of the substituted succinic anhydride of the present invention as a sizing agent or preferable operability in the acidic paper making step or neutral paper making step. The copolymerization is preferably aqueous soluble polymerization, and the molecular weight of the aqueous soluble copolymer (Aᵢ) is approx. 5,000 or more and more preferably 20,000 or more to be effectively used.

The aqueous soluble copolymer (A₂) preferably contains 70 percent or more by weight of the above mixture monomer ingredients and 30 percent or less by weight of other copolymer monomer as monomer ingredients, and can be readily produced similarly to the case of the aqueous soluble copolymer (A₁). This aqueous soluble copolymer (A₂) becomes preferable in the quality of the sizing agent when utilizing the aqueous dispersed solution of the substituted succinic anhydride of the present invention as sizing agent in the case where, similarly to the aqueous soluble copolymer (Aᵢ), regarding the (meth)acrylamide (a), N,N-dialkylaminoalkyl(meth)alkylamide (b) and (meth)acrylic acid (c), 75 to 94 percent by mol of (meth)acrylamide (a), 5 to 20 percent by mol of N,N-dialkylaminoalkyl(meth)acrylamide (b) and 1 to 10 percent by mol of (meth)acrylic acid (c) are contained. Further, the case of the aqueous soluble copolymer (A₂), containing 5,000 or more and more preferably having 20,000 or more of molecular weight is effectively used. Incidentally, as other copolymer monomer ingredients of 30 percent or less by weight of the copolymer (A) in the aqueous soluble copolymer (A₂), there are, for example, aromatic vinyl monomer such as styrene, alkylstyrene; alpha-, beta-unsaturated carboxylic acid esters such as alkylester, hydroxyalkylester, aminoalkylester of alpha-, beta-unsaturated carboxylic acid, vinyl acetate or other fatty acid vinylesters; other vinyl compounds such as vinylether or vinylamide; aryl compounds such as arylalcohol or arylether and arylamine or diarylamine and their quaternary ammonium salt; polymerizable quaternary ammonium compounds quaternarized from the N,N-dialkylaminoalkyl(meth)acrylamide, aminoalkyl-(meth)acrylate and vinylpyridine, or other polymerizable unsaturated compounds.

The contents of the substituted succinic anhydride in the aqueous dispersion of the substituted succinic anhydride according to the present invention can be arbitrary selected, but generally ranging from 0.01 percent by weight to 25 percent by weight to obtain stable aqueous dispersion. The aqueous dispersion of the present invention has particularly excellent utility in the stability at diluting time. If less than the concentration of less than 1 percent by weight, the effect performed by the diluting stability further becomes apparent.

The total amount of the contents of aqueous soluble copolymers (A₁) and (A₂) contained in the aqueous dispersed solution according to the present invention are generally preferably ranged from 0.05 percent by weight to 20 percent by weight, and the total of the aqueous soluble copolymers (A₁) and (A₂) is preferably selected in a range from about 0.2 to 2 parts by weight.

Further, the aqueous dispersed solution of the substituted succinic anhydride according to the present invention can, of course, additionally comprise other surfactants or aqueous soluble polymer substances. More specifically, when small amount of an oil-in-water type surfactant made, for example, of polyoxy- alkylenealkyl(aryl)ether and its sulfuric acid half ester or phosphoric acid ester, the dispersed particle diameter of the substituted succinic anhydride in the aqueous dispersion can be very finely pulverized, and the aqueous dispersed solution of the substituted succinic anhydride which additionally contain small amount of such oil-in-water type surfactant is most preferable for the aqueous dispersed solution of the present invention. In the aqueous dispersion containing the oil-in-water type surfactant, 0.1 to 10 percent by weight of oil-in-water type surfactant contained in the substituted succinic anhydride is ordinarily preferable.

The aqueous dispersed solution of the substituted succinic anhydride according to the present invention can be readily produced by adding a substituted succinic anhydride (B) to an aqueous solution which contains the aqueous soluble copolymer (Aᵢ) or (A₂), or both, and mechanically emulsifying and dispersing the mixture by various types of a homogenizer or a mixer. When a small amount of oil-in-water type surfactant is additionally employed, it is preferable to use the prepared mixture of the oil-in-water type surfactant and the substituent succinic anhydride (B). Incidentally, the oil-in-water type surfactant used for the prepared mixture may use any having mutual solubility with the substituted succinic anhydride (B), and it is preferable to selectively use the surfactant which provides excellent underwater dispersing ability in the substituted succinic anhydride (B) and less affects the adverse influence to the sizing effect such as, for example, polyoxyalkylenealkyl(aryl)ether and its sulfuric half-ester or phosphoric acid ester. The content of the oil-in-water type surfactant in the prepared mixture is preferably 0.1 to 10 percent by weight. More preferable oil-in-water type surfactant is a polyoxyalkylenealkyl(aryl)ether phosphoric acid ester represented by the following general formula where R₃ is an alkyl group or alkylaryl group having 8 or more carbon atoms, X represents an alkylene group, A represents a hydrogen or formula R'-(D-X)₁- (in the formula R' is an alkyl group or alkylacryl group, X represents an alkylene group, 1 represents an integer equal to or greater than 1), and m represents an integer equal to or greater than 1. This is particularly excellent in the solubility with the substituted succinic anhydride or underwater dispersibility of the substituted succinic anhydride. When the oil-in-water surfactant in which R₃ in the general formula is an alkyl group or alkylaryl group having 10 to 20 carbon atoms, X is an ethylene group, m is an integer equal to or greater than 5 is employed, the underwater dispersed particles of the substituted succinic anhydride produced by dispersing the mixture of the substituted succinic anhydride and the oil-in-water surfactant in the aqueous soluble compolymer (A,), the aqueous soluble copolymer (A₂) or in the aqueous solution of the both aqueous soluble copolymers become very ultrafine. When the sizing effect of the aqueous dispersed solution used as paper making sizing agent is furthger excellent, and becomes more preferable aqueous dispersed solution of the substituted succinic anhydride. To produce the aqueous dispersed solution of the substituted succinic anhydride according to one aspect of the present invention by employing the mixture of the substituted succinic anhydride (B) and the oil-in-water type surfactant, 1 part by weight of the mixture, and the aqueous solution containing 0.1 to 2 percent by weight of the aqueous soluble copolymer (A,) are mixed and agitated at arbitrary ratio. The agitator used in this case includes an ordinary propeller type agitator or other various homogenizer or a mixer.

The aqueous dispersed solution of the substituted succinic anhydride of the present invention as described above is mainly utilized as a paper making sizing agent, but may be utilized for a sizing agent in various fibrous industrial relations. Incidentally, in the utility as the paper making sizing agent, the aqueous dispersed solution of the substituted succinic anhydride is prepared in arbitrary or desired concentration, and can be applied to all paper making steps such as acidic paper making step using sulfuric acid band and neutral paper making step using no sulfuric acid band as sizing agent added to a pulp slurry as a paper making raw material or surface sizing agent to be coated by arbitrary means on wet or dry sheet after formed.

In the aqueous dispersed solution of the substituted succinic anhydride according to the present invention, the abovementioned aqueous soluble copolymer (A,) and the aqueous soluble copolymer (A₂) added and contained in the dispersed solution exhibit high adsorbility to pulp. Thus, the ultrafine substituted succinic anhydride particles in the dispersed solution can be efficiently adhered to the surface of the fiber of the pulp to perform the advantages of the present invention.

The underwater dispersibility of the aqueous soluble copolymers (A,) and (A₂) contained in the aqueous dispersed solution of the substituted succinic anhydride of the present invention for the substituted succinic anhydride is much superior to that of the copolymer of the (meth)acrylamide (a) and the N,N-dialkylaminoalkyl(meth)acrylamide (b), and such operations of the aqueous soluble copolymer (A,) and (A₂) provides extremely high dilute stability of the aqueous dispersed solution of the substituted succinic anhydride of the present invention.

Further, the aqueous soluble copolymers (A,) and (A₂) contained in the aqueous dispersed solution of the present invention are conducted in such a manner that the carboxyl group based on the (meth)acrylic acid monomer ingredient of the copolymer (A,) or (A₂) reacts with aluminum multi-valency cation in the sulfuric acid band. Consequently, when the aqueous dispersed solution of the substituted succinic anhydride according to the present invention is applied as paper making sizing agent, various troubles such as wires, roll and felts of the paper making machine to be contaminated in the paper making process can be avoided in addition to the excellent sizing effect.

### Examples and Comparison Examples

Parts by weight of the surfactants listed in the column of Table 1 were added to 100 parts by weight of alkenyl succinic anhydride, agitated and mixed at ambient temperature, and the composition of the alkenyl succinic anhydride was produced. The alkenyl succinic anhydride was produced by reacting inner olefin having 90 percent by weight of olefin having 15 to 18 carbon atoms and double bonds at 2 to 4 positions with maleic anhydride in accordance with the ordinary process.

Then, the composition of the alkenyl succinic anhydride was mixed similarly by parts in the solution of 10 percent by weight of aqueous soluble polymer compound listed in the columns of Table 1, agitated by a homogenization mixer (HV: M type produced by Tokushu Kika Kogyo K.K.) at 50 V for one minute, and the aqueous dispersed solutions of the substituted succinic anhydrides were prepared.

### Experiment 1

The aqueous dispersed solutions produced in the above examples and comparison examples were added to 2 percent by weight of pulp slurry (L-BKP, c.s.f.: 400 cc) containing 20 percent by weight of heavy calcium carbonate filler (Escaron # 800 produced by Sankyo Seifun K.K.) with respect to the weight of the pulp and similarly 1 percent by weight of pasted cationic starch with respect to the weight of the pulp so that the compositions of the substituted succinic anhydride and the surfactant in the aqueous dispersed solution became 0.15 percent by weight of the pulp, then, manual paper of the weight of 80 g/m² was prepared in accordance with the ordinary process with TAPPI Standard sheet machine, dried by a rotary drier at 110°C for 120 seconds, and manual paper was produced.

The produced paper was prepared in moisture and measured in accordance with JIS (the Japanese Industrial Standards) with respect to Stockigt sizing degree (sec) and listed in Table 2.

In Table 2, the emulsion mean particle diameters (pm) of the aqueous dispersed solution, the emulsion mean particle diameters (µm) of the dispersed solutions after allowed to stand for 10 hours, and the stabilize of the diluted dispersion diluted so that the composition of the alkenyl succinic anhydride and the surfactant became 0.05 percent by weight with civil water having 100 of total hardness in the dispersed solutions are listed.

### Experiment 2

The aqueous dispersed solutions produced in the above examples and comparison examples were added to 2 percent by weight of pulp slurry (L-BKP, c.s.f.: 400 cc) containing 20 percent by weight of talc with respect to the pulp weight and similarly 0.5 percent by weight of sulfuric acid band (Al₂(SO₄)₃ 16-18H₂0) with respect to the pulp weight so that the compositions of the substituted succinic anhydride and the surfactant in the aqueous dispersed solution became 0.2 percent by weight of the pulp, then similarly to the Experiment 1 to obtain paper. The produced paper was prepared in moisture and measured according to JIS (the Japanese Industrial Standards) with respect to stockist sizing degree (sec) and listed in Table 3.

### Experiment 3

The aqueous dispersed solutions produced by the examples and the comparison examples were added to pulp slurry produced with the same compositions as those used in the Experiment 2 so that the compositions of the substituted succinic anhydride and the surfactant in the aqueous dispersed solution became 1 percent by weight of the pulp weight, paper was made similarly to the Experiment 1, and wet sheet was prepared. The produced moistened sheet was interposed between a chromium plated plate and filter paper, pressed to remove water for 5 min under the pressure of 3.5 bar, the moistened sheet was then removed from the plate, and the contaminants on the surface of the plate were observed with bare eyes (presence of adhesive such as fine fiber). The results were listed in Table 4.

According to the present invention, the aqueous dispersed solution of the substituted succinic anhydride is as constituted and operated as described above, and the aqueous solution of the substituted succinic anhydride has the same diluted stability as the aqueous dispersion of the substituted succinic anhydride utilizing the conventional cationic starch by the stabilization of the aqueous soluble copolymer (A,) and/or the aqueous soluble copolymer (A₂) in the aqueous dispersed solution or in both the copolymers (A,) and (a₂), and provides the feasibility of handling in case of utilizing the emulsion particle size further finer than the emulsion particle size in the aqueous dispersed solution of the substituted succinic anhydride and industrial scale equivalent to those of the aqueous dispersion of the substituted succinic anhydride using the conventional synthetic polymer. Accordingly, when the aqueous dispersed solution of the substituted succinic anhydride is utilized as the sizing agent in paper making steps, the adition of the substituted succinic anhydride is very low such as 0.15 percent by weight with respect to the pulp weight, sufficiently satisfactory sizing agent can be produced.

Since the aqueous dispersed solution of the substituted succinic anhydride of the present invention has excellent fixing action to pulp fiber in the presence of sulfuric acid band, when the aqueous dispersed solution of the substituted succinic anhydride is used as paper making sizing agent, excellent sizing effect can be provided in all paper making steps including paper making stages using the sulfuric acid band. In addition, the paper making steps can be conducted without contamination of wires, rolls and other parts of the paper making machine to provide excellent operability.

## Claims

1. An aqueous dispersion of a substituted succinic anhydride comprising an aqueous soluble copolymer - or a mixture monomer ingredient in an aqueous soluble copolymer - which has 50 percent or more by mol of (meth)acrylamide, 1 per cent or more by mol of N,N-dialkylaminoalkyl(meth)acrylamide, and a quantity of (meth)acrylic acid, characterised in that the first-mentioned coploymer or the mixture monomer ingredient has up to 98.5 percent by mol of (meth)acrylamide, up to 49.5 percent by mol of N,N-dialkylaminoalkyl(meth)acrylamide, and from 0.5 to 20 per cent by mol of (meth)acrylic acid.

2. An aqueous dispersion of a substituted succinic anhydride comprising an aqueous soluble copolymer with a mixture monomer ingredient according to claim 1, characterised in that the copolymer contains 70 percent or more by weight of the mixture monomer ingredient.

3. An aqueous dispersion of a substituted succinic anhydride according to claim 2, characterised in that the two forms of copolymer are both present in the dispersion.

4. An aqueous dispersion of a substituted succinic anhydride according to any one of claims 1-3, characterised in that the first-mentioned copolymer, or each copolymer, contains 75 to 94 per cent by mol of (meth)acrylamide, 5to 20 per cent by mol of N,N-dialkylaminoalkyl(meth)acrylamide, and 1 to 10 percent by mol of (meth)acrylic acid.

5. An aqueous dispersion of a substituted succinic anhydride according to any one of claims 1-4, characterised in that the substituted succinic anhydride is an alkenyl succinic anhydride.

6. An aqueous dispersion of a substituted succinic anhydride according to any one of claims 1-5, characterised in that oil-in-water type surfactant is contained as a dispersing aid.

7. An aqueous dispersion of a substituted succinic anhydride according to claim 6, characterised in that the oil-in-water type surfactant is polyoxyalkylene alkyl(aryl)ether phosphoric acid ester.

## Patentansprüche

1. Wäßrige Dispersion eines substituierten Bernsteinsäureanhydrids umfassend ein wasserlösliches Copolymer- oder eine Mischung von Monomerbestandteilen in einem wasserlöslichen Copolymer-, welches 50 Mol-% oder mehr (meth)Acrylamid, 1 Mol-% oder mehr N,N-Dialkylaminoalkyl(meth)acrylamid und eine Menge an (meth)Acrylsäure enthält, dadurch gekennzeichnet, daß das esterwähnte Copolymer oder die Mischung von Monomerbestandteilen bis zu 98,5 Mol-% (meth)Acrylamid, bis 49,5 Mol-% N,N-Dialkylaminoalkyl(meth)acrylamid und von 0,5 bis 20 Mol-% (meth)Acrylsäure enthält.

2. Wäßrige Dispersion eines substituierten Bernsteinsäureanhydrids umfassend ein wasserlösliches Copolymer mit einer Mischung von Monomerbestandteilen gemäß Anspruch 1, dadurch gekennzeichnet, daß das Copolymer 70% oder mehr der Mischung an Monomerbestandteilen enthält.

3. Wäßrige Dispersion eines substituierten Bernsteinsäureanhydrids gemäß Anspruch 2, dadurch gekennzeichnet, daß die beiden Formen des Copolymers in der Dispersion vorliegen.

4. Wäßrige Dispersion eines substituierten Bernsteinsäureanhydrids gemäß einem der Ansprüche 1 bis 3, dadurch gekennzeichnet, daß das ersterwähnte Copolymer, oder jedes Copolymer, 75 bis 94 Mol-% (meth)Acrylamid, 5 bis 20 Mol-% N-N-Dialkylaminoalkyl(meth)acrylamid, und 1 bis 10 Mol-% (meth)Acrylsäure enthält.

5. Wäßrige Dispersion eines substituierten Bernsteinsäureanhydrids gemäß einem der Ansprüche 1 bis 4, dadurch gekennzeichnet, daß das substituierte Bernsteinsäureanhydrid ein Alkenylbernsteinsäureanhydrid ist.

6. Wäßrige Dispersion eines substituierten Bernsteinsäureanhydrids gemäß einem der Ansprüche 1 bis 5, dadurch gekennzeichnet, daß ein Öl-in-Wasser-oberflächenaktives Mittel als Dispergierhilfe enthalten ist.

7. Wäßrige Dispersion eines substituierten Bernsteinsäureanhydrids gemäß Anspruch 6, dadurch gekennzeichnet, daß das Öl-in-Wasser-oberflächenaktive Mittel Polyoxyalkylenalkyl(aryl)ether-Phosphorsäureester ist.

## Revendications

1. Dispersion aqueuse d'un anhydride succinique substitué, comprenant un copolymère soluble aqueux - ou un ingrédient monomérique en mélange dans un copolymère soluble aqueux qui contient 50 ou plus de 50%, en moles, de (méth)acrylaide, 1% ou plus de 1%, en moles, de N,N-dialkylaminoalkyl(méth)acrylamide et une quantité d'acide (méth)acrylique, caractérisée en ce que le copolymère mentionné en premier lieu ou l'ingrédient monomérique en mélange contient jusqu'à 98,5%, en moles, de (méth)acrylamide, jusqu'à 49,5%, en moles, de N,N-dialkylaminoalkyl(méth)acrylamide et 0,5 à 20%, en moles, d'acide (méth)acrylique.

2. Dispersion aqueuse d'un anhyride succinique substitué comprenant un copolymère soluble aqueux avec un ingrédient monomérique en mélange selon la revendication 1, caractérisée en ce que le copolymère contient 70 ou plus de 70% en poids de l'ingrédient monomérique en mélange.

3. Dispersion aqueuse d'un anhyride succinique substitué suivant la revendication 2, caractérisée en ce que les deux formes de copolymère sont toutes deux présentes dans la dispersion.

4. Dispersion aqueuse d'un anhyride succinique substitué suivant l'une quelconque des revendications 1 à 3, caractérisée en ce que le copolymère mentionné en premier lieu ou chaque compolymère contient 75 à 94%, en moles, de (méth)acrylamide, 5 à 20%, en moles, de N,N-dialkylaminoalkyl(méth)acrylamide et 1 à 10%, en moles, d'acide (méth)acrylique.

5. Dispersion aqueuse d'un anhyride succinique substitué suivant l'une quelconque des revendications 1 à 4, caractérisé en ce que l'anhydride succinique substitué est un anhydride alcénylsuffinique.

6. Dispersion aqueuse d'un anhyride succinique substitué suivant l'une quelconque des revendications 1 à 5, caractérisée en ce qu'un surfactant du type huile-dans-eau est contenu comme substance auxiliaire de dispersion.

7. Dispersion aqueuse d'un anhyride succinique substitué suivant la revendication 6, caractérisée en ce que le surfactant du type huile-dans-eau est un ester d'acide polyoxyalkylène-alkyl(aryl)éther- phosphorique.
